

# UNITED STATES PATENT OFFICE.

WILLIAM A. MCADAMS, OF BAY SHORE, NEW YORK.

## ALUMINUM ALLOY.

1,099,561.

Specification of Letters Patent.

Patented June 9, 1914.

No Drawing.

Application filed February 11, 1913. Serial No. 747,671.

*To all whom it may concern:*

Be it known that I, WILLIAM A. MCADAMS, a citizen of the United States, and resident of Bay Shore, in the county of Suffolk and State of New York, have invented a new and useful Aluminum Alloy, of which the following is a specification.

My invention relates to an aluminum alloy with the object in view of providing an inexpensive alloy which can be readily rolled into thin sheets; which will not tarnish and which will have a fair degree of stiffness and resiliency.

With these ends in view, my invention consists in an alloy composed of aluminum, copper and silver in which the amount of aluminum exceeds the amount of copper and the amount of copper exceeds the amount of silver. More particularly, the aforesaid elements are preferably combined in the proportion of one hundred parts by weight of aluminum, five parts by weight of copper and two parts by weight of silver.

In making the alloy, the aluminum is preferably first melted and the copper and silver introduced into the melted aluminum and the mass raised to such a degree as to melt the copper and silver, the melted mass being thoroughly agitated to bring the molecules of the different elements into intimate contact. The mass is then allowed to cool, and may then be rolled or tooled as may be desired. When rolled into a thin sheet, the alloy will present a brilliant white surface which will not tarnish; the sheet may be

bent at pleasure, and will be so stiff and hard and at the same time resilient that the metal will keep the form into which it is bent without liability of becoming mashed out of shape. The small proportion of silver relative to the amount of copper and the small proportion of both silver and copper relative to the amount of aluminum makes the alloy almost as light as aluminum itself and adds but little to the cost of the alloy over the cost of aluminum alone.

I am aware that the elements, aluminum, copper and silver have heretofore been combined to form an alloy in which the silver exceeded the copper, but I believe that I am the first to succeed in producing a non-tarnishable, tough, resilient and stiff alloy capable of being rolled and worked like silver or copper by using an amount of silver so relatively small as compared with the amount of copper and aluminum.

What I claim is:

An aluminum alloy composed of aluminum, copper and silver combined substantially in the proportions of one hundred parts aluminum, five parts copper and two parts silver.

In testimony that I claim the foregoing as my invention, I have signed my name in presence of two witnesses, this twenty-third day of January, 1913.

WILLIAM A. MCADAMS.

Witnesses:

F. GEORGE BARRY,  
HENRY C. THIEME.